

## UNITED STATES PATENT OFFICE

EDWIN C. WALLACE, OF NEWTON, MASSACHUSETTS

## ROAD MAKING AND MATERIAL USED THEREIN

No Drawing.

Application filed July 2, 1928. Serial No. 290,052.

The present invention relates to the manufacture of roads (under which term I intend to embrace not only ordinary roadways for open vehicular traffic, but also walks, paths, roofs, etc.) and also embraces a novel composition of matter the use of which constitutes an essential feature of such manufacture.

Many rocks found in various parts of the world are more or less thoroughly impregnated with bitumen. Some of these, Neufchateau, val de Travers, and Ragussa or Sicilian rock, have been extensively used for various purposes such as roofs, floors, sidewalks and street paving work, with excellent results. Investigation has shown that the bitumen with which all of this rock is impregnated is of very soft consistency.

Many other rocks are found in which the impregnating bitumen is of much harder consistency than in the rocks mentioned above. Many attempts have been made to use the kinds of rock impregnated with hard bitumen, in road making with results which are extremely variable and wholly uncertain. Fairly good results have been obtained in some cases when efforts were made to soften the bitumen with which the rock was impregnated by the addition of a suitable flux or softening agent. By this means compositions were sometimes produced which gave excellent results, but quite different and unsatisfactory results were so frequently obtained that attempts have been made to overcome the difficulty.

In some of these attempts the methods outlined have been so very elaborate as to be suitable only for the laboratory or small scale production.

In the process herein described an attempt has been made to soften the bitumen contained in the rock by the addition, in a specific manner described below, of suitable fluxing or softening agent of the same general character which has been proposed, but the method has been so modified that uniformly good results may be obtained without the necessity of carrying the refinements beyond the limits of practicability from the standpoint of cost.

In this process it is not necessary to heat the asphalt rock and except in cases where

heavy gravity, viscous fluxes are used it is not necessary to heat the flux. Where, however, a heavy gravity and viscous flux is used, it is advisable to heat it to somewhat above the boiling point of water before it is added to the rock asphalt.

In brief, the process may be described as follows:

The asphalt rock is broken into fragments which will pass a screen, the openings of which will give particles of the maximum size desired. The reduced material is then separated by screens into two portions, one much finer than the other.

These sizes may vary according to the purpose for which the composition is to be used, but as examples of material suitable in most cases, the following may be given:

The rock may be crushed into sizes substantially all of which will pass a screen having  $\frac{3}{4}$  inch or  $\frac{1}{2}$  inch openings and the fine material which passes an 8-10 mesh screen, is then kept separated from the portion retained thereon. This forms two fractions, a coarse fraction and a fine fraction.

The approximate proportion of coarse to fine material obtained by crushing and screening, is noted in order that these materials may be recombined later in substantially the same ratio.

After the crushed rock has been separated as described, the coarse material is introduced into any suitable mixing device and to it the necessary proportion of fluxing or softening agent is added and these ingredients then thoroughly mixed. The finer material obtained by screening as above is thereafter added and the entire mass thoroughly commingled.

The proportions of coarse and fine crushed rock may be varied at will, but by using it in substantially the same proportions into which the rock breaks down, there is no excess of either coarse or fine and no loss of material.

The amount of flux or softening agent will vary with its viscosity but generally comes within the limits of 1 to 4% by weight of the rock which would be approximately equal to 3 to 10 gallons of flux to each ton of crushed rock.

Any suitable flux for asphalt may be used, but I prefer one derived from Mexican or California petroleum and also by preference use one having a viscosity of less than 2000 seconds on Engler viscosimeter at 25° C., with specific gravity coming within a range of .82 to .96 at 25° C.

With this relatively small proportion of softening agent, it is essential that proper distribution be obtained.

By separating the crushed rock into coarse and fine fractions and applying the fluxing material to the coarse material only, the component pieces in this fraction become thoroughly coated with the flux and act as a dispersing medium to distribute said fluxing material to and through the finer fraction, during the subsequent mixing and compression operations. The flux-treated coarse material is mixed with the fines in their original ratio.

Each of the flux-coated coarse pieces becomes in effect a nucleus around which the finer particles accrete and become coated by contact and diffusion.

This mixture is then spread on the foundation, preferably at atmospheric temperature, to the desired thickness and rolled or otherwise compressed and compacted to form a road, walk or other desired article.

If it were attempted to mix the whole of the coarse and fine (without separation) directly with this small amount of flux, or if it were attempted to mix the fine material with this small amount of flux and subsequently incorporate the coarser material, the flux or softening agent would come into contact with the finer material before the coarse particles would be properly coated and the fine material would act as a sponge or absorbent, and take up much more of the fluxing agent than is actually needed by it, and render it practically impossible to distribute the small amount of flux required, uniformly through the mass. The final result would be an improperly balanced composition much richer and softer in some portions than in others. If the softer portions richer in the fluxing material are well adapted for the purpose for which the composition is to be used, the drier, harder portions containing a smaller percentage of flux can not be; conversely if the dry, hard portions are suitable the softer, richer portions are not. Under such conditions satisfactory results are not to be expected.

By the method herein described this difficulty is overcome, the finer material does not carry more than its proportionate share of the fluxing agent, the composition is properly balanced, easily controlled and excellent and uniform results can be obtained.

I claim:—

1. In the preparation of bituminous paving mixtures from rock asphalt impregnated

with hard bitumen, the successive steps of crushing the rock asphalt to a desired size, separating it into two portions of respectively coarse and fine particles, mixing the coarse portion with a small amount of asphalt fluxing or softening agent, then recombining the coarse and fine material in substantially the proportions in which the rock breaks down.

2. A process which comprises crushing a rock containing hard asphalt, until all of the rock will pass a screen of  $\frac{3}{4}$  inch mesh, then screening out the fine material from the coarser material contained therein, well mixing the coarser portion with about 1 to 4% of fluxing oil, thereafter adding the finer material, in about the proportions into which the coarse and fine portions were originally separated.

In testimony whereof I affix my signature.

EDWIN C. WALLACE.

85

90

95

100

105

110

115

120

125

130